

No. 818,415.

PATENTED APR. 24, 1906.

G. F. COLE.  
HEAT RESISTING FABRIC.  
APPLICATION FILED FEB. 20, 1905.



Witnesses.

Edward L. Hill  
A. O. Bement

Inventor,

Giles F. Cole  
per Clark C. Merritt

Attorney.

# UNITED STATES PATENT OFFICE.

GILES F. COLE, OF LANSING, MICHIGAN.

## HEAT-RESISTING FABRIC.

No. 818,415.

Specification of Letters Patent.

Patented April 24, 1906.

Application filed February 20, 1905. Serial No. 246,390.

*To all whom it may concern:*

Be it known that I, GILES F. COLE, a citizen of the United States, residing at Lansing, in the county of Ingham and State of Michigan, have invented a new and useful Improvement in Heat-Resisting Fabrics, of which the following is a specification.

My invention relates to heat-resisting fabrics; and the purpose of the invention is to make a fabric which shall be soft and pliable in its texture, not likely to scratch or injure any varnished surface upon which it may be laid, cheap in construction, and durable and effective for the purpose for which it is intended.

The figure shows a piece of my fabric having the three layers separated at one end to show the construction.

A and C are layers of some textile fabric, preferably canton-flannel or some similar fabric having soft and fleecy exterior surfaces.

B is a layer of asbestos fabric softened and made pliable and cemented between the two layers A and C, so as to form one compound fabric which is nearly as pliable as if it were formed entirely of cloth, the soft and fleecy character of the outside layers, combined with the heat-resisting qualities of the asbestos center, making the fabric extremely effective when used as a table-covering or in other places where it is desired to exclude heat. Moreover, its composition is such that it can be made up and sold in large bolts or rolls,

like ordinary cloth, and can be cut and sewed or fashioned in any shape or manner in which ordinary cloth can be employed.

I am aware that asbestos has been often used in combination with other substances as a heat-resisting medium; so I do not broadly claim this.

What I do claim as a new article of manufacture is—

1. A compound fabric composed of a softened flexible sheet of asbestos fiber cemented between two layers of textile fabric having a fleecy exterior surface.

2. A compound fabric composed of a softened flexible sheet of asbestos fiber cemented between two layers of textile fabric having fleecy surfaces.

3. A compound heat-resisting fabric composed of a softened flexible sheet of asbestos fiber cemented between two layers of canton-flannel, the fleecy side of said flannel being out.

4. A compound heat-resisting fabric composed of a softened flexible sheet of asbestos fiber cemented between two layers of two-faced canton-flannel.

In testimony whereof I have signed my name to this specification in the presence of two subscribing witnesses.

GILES F. COLE.

Witnesses:

H. L. LAWRENCE,  
C. C. Wood.